

## UNITED STATES PATENT OFFICE

2,210,595

## AQUEOUS TEXTILE FIBER IMPREGNATING COMPOSITION

Max Nassau, Berlin-Wilmersdorf, Fritz Sommer, Berlin-Charlottenburg, and Georg Wiegand, Berlin-Grunau, Germany, assignors to the firm: Chemische Fabrik Grunau Landshoff & Meyer A. G., Berlin-Grunau, Germany, a company of Germany

No Drawing. Application May 3, 1937, Serial No. 140,450. In Germany September 6, 1933

6 Claims. (Cl. 134—11)

This invention relates to an improvement in an aqueous textile fiber impregnating composition.

It is known, in the manufacture of water-repellent textile fabrics and related products by impregnation processes, to employ dispersions of fatty substances containing aluminium salts. According to the older methods for waterproofing textile products the fabrics to be impregnated were treated first with aluminium salts and then with an aqueous dispersion of the fatty substance. That process using two baths successively was comparatively inconvenient and expensive.

When using dispersions of fatty substances containing aluminium salts, a single bath proved sufficient for impregnating textile products. However, the aluminium salts having a flocculating effect upon the dispersions of the fatty substances, it became necessary to add protective colloids to said dispersions in order to prevent flocculation. As protective colloids there have been used mainly glue, gelatine, and tragacanth. These protective colloids effect a kind of congealing of the dispersion, i. e. a solidification of the entire dispersion whereby flocculation will be prevented. These congealed dispersions are referred to as "dead" dispersions and require re-melting prior to being used. Furthermore, dispersions containing protective colloids are not capable of being readily used in all cases, the protective colloids mentioned above imparting an undesirable hard feel to the treated vegetable and animal fibres.

It is the general object of the present invention to remove all these disadvantages. A more specific object is dispersions of fatty substances containing aluminium salts which are stable, i. e. do not flocculate and are not affected by the hardening constituents of water. A still further object is dispersions of fatty substances containing aluminium salts which when used for impregnating textile products will make said products waterproof without affecting their natural feel.

These objects are accomplished by incorporating with the dispersions, in addition to aluminium salts, the condensation products of high molecular split-off products of albumin of the lysalbinic and protalbinic acid type with higher fatty acid chlorides. These condensation products are obtained by reacting high molecular split-off products of the lysalbinic and protalbinic acid type with higher fatty acid chlorides in an alkaline solution, as described in

U. S. patent to Fritz Sommer, No. 2,015,912. Precipitation of the condensation products is effected by adding an acid to the solution. The dispersions to be used for impregnating purposes are prepared by reacting these condensation products with aluminium salts. The dispersions so obtained are able to disperse still further amounts of fatty substances of various kinds, such as paraffin wax. These dispersions containing additional fatty substances will give particularly desirable impregnating effects.

Our invention is illustrated but not limited by the following examples in which parts are by weight.

## Example I

15

81 parts of a solution of high molecular split-off products of albumin which has been prepared by alkaline decomposition of leather waste, are reacted with 18 parts of stearic acid chloride the solution being kept alkaline by means of caustic soda. A solution of sodium stearyl lysalbinic acid is thus obtained. By adding a mineral acid to the solution stearyl lysalbinic acid is precipitated.

150 parts of the isolated stearyl lysalbinic acid are stirred with 500 parts of an aluminium formate solution of 15% till a homogeneous dispersion has been formed. For impregnating purposes the dispersion so obtained is being diluted in the ratio of 1:25. Textile fabrics treated with this solution are made water-repellent without acquiring a hard feel.

## Example II

35

To 650 parts of the dispersion prepared according to Example I there are added, at 60° to 70° C., 250 parts of melted paraffin wax. The mixture is stirred till a homogeneous salve-like mass has been formed. Even when stored for a prolonged time this salve-like mass is stable, i. e. no separation of the phases will occur. For impregnating purposes this salve-like mass is being diluted in the ratio of 1:100. When used for treating textile products this dispersion is particularly effective in making the products waterproof without affecting their natural feel.

Instead of aluminium formate named in the examples, there may be employed various other aluminium salts such as aluminium acetate, aluminium sulphate, soda alum, potash alum, and ammonia alum, as will be obvious to those familiar with the art.

Similarly, as an alternative to stearyl lysalbinic acid, there may be used other condensation prod-

55

ucts of higher fatty acid chlorides with high molecular split-off products of albumin such as oleyl lysalbinic acid.

Furthermore, other fatty substances such as saponifiable fats or waxes may be substituted for paraffin wax.

We claim:

1. An aqueous textile fiber impregnating composition comprising an aqueous dilute dispersion of the reaction product of a higher fatty acid substituted lysalbinic acid with an aluminum salt in water solution, said reaction product being present in the composition in sufficient amount to impart to textile fibers treated therewith water-repellant properties.

15 2. An aqueous textile fiber impregnating composition comprising an aqueous dilute dispersion of the reaction product of a higher fatty acid substituted lysalbinic acid with an aluminum salt in water solution, said composition having incorporated therein a substantial quantity of wax, said reaction product being present in the composition in sufficient amount to impart to textile fibers treated therewith water-repellant properties.

25 3. An aqueous textile fiber impregnating composition comprising an aqueous dilute dispersion of the reaction product of a stearyl lysalbinic acid with an aluminum salt in water solution, said reaction product being present in the composition in sufficient amount to impart to textile fibers treated therewith water-repellant properties.

4. An aqueous textile fiber impregnating composition comprising an aqueous dilute dispersion of the reaction product of an oleyl lysalbinic acid with an aluminum salt in water solution, said reaction product being present in the composition in sufficient amount to impart to textile fibers treated therewith water-repellant properties.

5 5. An aqueous textile fiber impregnating composition comprising an aqueous dilute dispersion of the reaction product of a higher unsaturated 10 fatty acid chloride and the high molecular split-off products of albumen of the lysalbinic and protalbinic acid type with an aluminum salt, said reaction product being present in the composition in sufficient amount to impart to textile fibers 15 treated therewith water-repellant properties.

6. An aqueous textile fiber impregnating composition comprising an aqueous dilute dispersion of the reaction product of a higher unsaturated 20 fatty acid chloride and the high molecular split-off products of albumen of the lysalbinic and protalbinic acid type with an aluminum salt, said reaction product being present in the composition in sufficient amount to impart to textile 25 fibers treated therewith water-repellant properties, said composition containing substantial amounts of paraffin wax, saponifiable fats and waxes.

MAX NASSAU.  
FRITZ SOMMER.  
GEORG WIEGAND.

30